

## UNITED STATES PATENT OFFICE

ARTHUR SCOTT SHOFFSTALL, WILLIAM ALVIN MUDGE, AARON BYSAR BAGSAR, AND CLARENCE GEORGE BIEBER, OF HUNTINGTON, WEST VIRGINIA, ASSIGNEES, BY MESNE ASSIGNMENTS, TO THE INTERNATIONAL NICKEL COMPANY, INC., OF NEW YORK, N. Y., A CORPORATION OF DELAWARE

## DESULPHURIZING NICKEL-CONTAINING MATTE

No Drawing.

Application filed May 3, 1928. Serial No. 274,963.

This invention relates to the Bessemerizing of nickel-containing mattes to desulphurize and deoxidize such mattes and produce metallic nickel or alloy containing nickel; and particularly to the blowing of nickel mattes and nickel-copper mattes, such as "Monel metal" mattes.

We are familiar with the work done by Otto Lellep in this art, and some of his inventions are described and claimed in Lellep Patents 1,599,424 and 1,623,797. While the Lellep process will produce metallic nickel from nickel mattes, it requires such high temperatures that the converter linings are 10 strongly attacked. We have discovered an improved process of Bessemerizing of nickel-containing mattes which has advantages over other Bessemerizing processes, such as the Lellep process, in that it permits of carrying 15 out desulphurization and deoxidation by blowing in a shorter time, and with the use of less expensive refractory materials for the converter linings. In our process the converter linings need be much less expensive, 20 and much longer life of the lining is secured, thereby materially reducing the cost of the process.

In carrying out our process in its preferred form, the nickel matte or nickel-containing matte, such as Monel metal matte, is charged into a converter in lump or ground up form. Such matte is melted in the converter furnace, preferably by the aid of gas blast burners, and the temperature of the molten matte is raised to about 2500° F. During this period, there is preferably no blowing. The molten matte at this stage ordinarily contains about 18% to 20% of sulphur.

When the temperature of the molten matte has been raised to about 2400-2700° F. and preferably between 2450° and 2650° F., superheated steam is forced into or in contact with the molten bath, this steam preferably having a relatively small amount of air mixed with it. The preferred mixture is about 90% of steam and about 10% of air by volume. This mixture is blown through the tuyères and the converter is tilted into the blow position where the superheated steam or the superheated steam-and-air blast preferably

passes directly through the molten matte. The burners projecting into the converter above the bath are then regulated so as to maintain the temperature of the bath from about 2450° F. to about 2650° F. Preferably samples are taken from the furnace every fifteen or twenty minutes during the blow to ascertain the sulphur content and find the amount of reduction thereof. The steam and air blast is continued within this temperature range until the samples show that the sulphur content of the melt has been lowered to about 2 to 4%. This constitutes the first stage of the process.

In the next stage the burners are regulated to raise the temperature to from 2700-2900° and preferably to about 2750 to 2850° F., and superheated steam alone is blown through the bath until the sulphur is practically eliminated. This may be ascertained by sampling the gases passing off, the substantial absence of sulphur dioxide in these gases being taken as evidence of substantially complete sulphur removal. During this second stage of sulphur elimination, the air is omitted in the blast so as to prevent its reacting with the metal to form metallic oxides instead of reacting with the sulphur in the bath. During this second blowing period, the sulphur content of the melt is preferably lowered from its content of from 2 to 4% down to a content ranging usually from .005 to .02%.

At the end of the second stage, the bath usually contains some oxygen in the form of oxides. This oxygen may be reduced or substantially eliminated from the metal by poling, by the use of a reducing flame, by carbon, or by any other suitable deoxidizing agent, such as magnesium, manganese, silicon, calcium, boron, etc. The deoxidation of the charge may be carried out either in the desulphurizing converter or furnace or in a second furnace or in a ladle or any suitable receptacle.

The above process requires much less time than the Lellep process, and there is far less corrosive effect on the lining. Ordinary medium priced refractory material may be used for the lining. Monel metal matte and

55

60

65

70

75

80

85

90

95

100

nickel sulphide mattes are very corrosive to refractory materials at temperatures higher than about 2650° F. but have very little destructive effect up to this temperature. When 5 the sulphur has been reduced to around 2 to 4%, the corrosive effect is largely eliminated. Hence, by blowing at a lower temperature for the first portion of the blow, and until the sulphur is considerably reduced, the corrosive effect 10 may be largely done away with, enabling a medium priced refractory to be used which will give a relatively large number of heats.

The first stage of the blow may be carried out by the use of superheated steam alone, 15 such steam being preferably at a temperature of from 800° F. to 1200° F., but the use of a certain percentage of air in this stage aids in the rapidity of sulphur removal and does not deleteriously affect the metal. Within the 20 lower temperature range, the steam-air mixture reacts with the sulphides more rapidly than steam alone, although steam alone may be used; but during the later stage of blowing the air should be substantially eliminated. 25 When blowing Monel metal mattes (nickel-copper), the temperature of the first stage may be slightly lower than that for nickel mattes.

One of the products of the reaction is hydrogen sulphide and the faster this gas is removed from the zone of reaction as it is formed, the faster will be the operation. The air aids in carrying off and burning the hydrogen sulphide as formed. The burning of 30 the sulphide with the air probably forms sulphur dioxide and steam. This active (nascent) steam generated by the oxidation of the H<sub>2</sub>S also serves to decompose additional 35 quantities of sulphide and reduce the time 40 of blowing.

Special forms of converters may aid in reducing or doing away with the need for air, especially such as will allow for rapid removal of the H<sub>2</sub>S. The steam is preferably 45 superheated to somewhere around 1000° F. before blowing it into the bath. Provided the temperature of the bath is held at a point somewhat below 2650° F., the rate of sulphur 50 elimination is believed to be directly proportional to the amount of desulphurization gas passed or blown through the molten material.

Instead of using burners such as natural gas blast burners above the level of the bath in the converter for melting and preheating 55 the charge before blowing and for raising the temperature in the second stage, the operation may be carried out in a suitably designed arc, resistor or induction electric furnace, provided with tuyères. In such case, 60 the electric current may supply the additional heat for obtaining the desired preliminary and final temperatures or any other way of adding heat units may be used as desired. For example, a combustible material may be 65 mixed with the steam and air blast, sufficient

air being employed to burn the combustible, this combustible being, of course, regulated to maintain the desired temperature of the first stage and also that of the second stage.

The temperature ranges above recited may be varied, the composition of the desulphurizing gas used may be changed, various types of furnaces may be used, the operation may be carried out on any nickel-containing matte, and other changes may be made without departing from our invention. 75

We claim:—

1. In the Bessemerizing of a nickel-containing matte or material, the step consisting of blowing with a desulphurizing gaseous 80 blast of which superheated steam forms the major portion.

2. In the Bessemerizing of a nickel-containing matte or material, the steps consisting of blowing a matte with a gaseous blast 85 through an earlier stage in which a major percentage of sulphur is removed, holding the bath during this stage at a temperature of from 2400 to 2700° F., and then raising the temperature to a range between 2700 and 90 2900° F. and continuing the blowing operation.

3. In the Bessemerizing of a nickel-containing matte or material, the steps consisting of forcing a gaseous blast in contact with the matte at a temperature of between 2400 and 2700° F., the blast containing steam as the major ingredient, and thereafter raising the temperature and blowing the same with steam in the substantial absence of air in 100 the blast.

4. In the Bessemerizing of a nickel-containing matte or material, the steps consisting of blowing the same with a mixture of steam and air in which air is the minor ingredient, at a temperature of from 2400 to 105 2700° F. and then raising the temperature to a point below 2900° F., and continuing the operation with steam which is substantially free from air.

5. In the Bessemerizing of a nickel-containing matte or material, the steps consisting of blowing the same with a blast containing steam and at a temperature below 110 2700° F. and above 2000° F., until the sulphur content is lowered to about 2 to 4% and then raising the bath to a higher temperature below 2900° F., and continuing the blowing with a blast substantially free from 115 free oxygen.

6. In the Bessemerizing of a nickel-containing matte or material, the steps consisting of heating the bath to a temperature between 2400° to 2700° F., blowing the same with a blast containing superheated steam, raising the temperature by applied heat until the bath is between 2700° to 2900° F., and continuing the blow with superheated steam 120 substantially free from free air.

7. In the Bessemerizing of a nickel-con-

taining matte or material, the steps consisting of blowing the bath with a steam-air mixture at a lower temperature above 2000° F., and then raising the temperature by applied heat and increasing the percentage of steam in the blast.

8. In the Bessemerizing of a nickel-containing matte or material, the steps consisting of blowing the same with a blast containing steam at a temperature below about 2700° F. and above 2000° F., then raising the temperature by applied heat and blowing with a blast containing a larger amount of steam at a higher temperature below about 2900° F., and then deoxidizing the metal.

9. In the desulphurizing of a nickel-containing matte or material, the steps consisting in bringing into contact with the matte at a suitable temperature, a mixture of steam and air in which the steam is the major ingredient.

10. In the Bessemerizing of a nickel-containing matte or material, the step consisting of blowing the same with a gaseous blast of which superheated steam having a temperature materially below that of the flaming arc forms the major portion.

11. In the Bessemerizing of a nickel-containing matte or material, the step consisting of blowing the same with a gaseous blast of which superheated steam at a temperature of from 800° to 1200° F. forms the major portion.

12. In testimony whereof we have hereunto set our hands.

ARTHUR SCOTT SHOFFSTALL.

WILLIAM ALVIN MUDGE.

AARON BYSAR BAGSAR.

CLARENCE GEORGE BIEBER.

40

45

50

55

60